



US005325922A

**United States Patent [19]**

Cowan et al.

[11] Patent Number: **5,325,922**[45] Date of Patent: **Jul. 5, 1994**

## [54] RESTORING LOST CIRCULATION

[75] Inventors: M. Kenneth Cowan, Sugar Land; Arthur H. Hale, Houston, both of Tex.

[73] Assignee: Shell Oil Company, Houston, Tex.

[21] Appl. No.: **964,819**[22] Filed: **Oct. 22, 1992**[51] Int. Cl.<sup>5</sup> ..... **E21B 33/13**[52] U.S. Cl. ..... **166/293; 166/292; 166/295; 175/72**[58] Field of Search ..... **166/292, 293, 294, 295; 175/64, 65, 66, 72; 507/140**

## [56] References Cited

## U.S. PATENT DOCUMENTS

- 2,336,723 12/1943 Drummond .  
 2,649,160 8/1953 Williams et al. .  
 2,776,112 1/1957 Ilfrey et al. ..... 175/64 X  
 2,822,873 2/1958 Harmsen et al. .  
 2,868,294 1/1959 Beale, Jr. et al. ..... 166/292  
 2,880,096 3/1959 Hurley .  
 2,895,301 7/1959 Casagrande et al. .  
 2,899,329 8/1959 Lyons .  
 2,961,044 11/1960 Shell .  
 2,983,353 3/1960 Vorenkamp .  
 3,021,680 2/1962 Hayward .  
 3,077,740 2/1963 Hemwall .  
 3,111,006 11/1963 Caron .  
 3,168,139 2/1965 Kennedy et al. .  
 3,412,564 11/1968 McClintock .  
 3,499,491 3/1970 Wyant et al. .  
 3,557,876 1/1971 Tragesser .  
 3,670,832 6/1972 Striegler .  
 3,675,728 7/1972 Faulk et al. .  
 3,712,393 1/1973 Sheldahl et al. .  
 3,724,562 4/1973 Striegler .  
 3,820,611 6/1974 King .  
 3,835,939 9/1974 McEntire .  
 3,887,009 6/1975 Miller et al. .  
 3,962,878 6/1976 Hansen .  
 3,964,921 6/1976 Persinski et al. .  
 4,014,174 3/1977 Mondshine .  
 4,037,424 7/1977 Anders .  
 4,057,116 11/1977 Striegler .  
 4,215,952 8/1980 Baardsen .  
 4,252,471 2/1981 Straub .  
 4,335,980 6/1982 DePriester .  
 4,338,134 7/1982 Graf zu Munster .  
 4,425,055 1/1984 Tiedemann .  
 4,427,320 1/1984 Bhula .  
 4,450,009 5/1984 Childs et al. .  
 4,460,292 7/1984 Durham et al. .  
 4,518,508 5/1985 Conner ..... 210/751  
 4,643,617 2/1987 Kanno et al. ..... 405/222  
 4,664,843 5/1987 Burba, III et al. .  
 4,668,128 5/1987 Hartley et al. .  
 4,674,574 6/1987 Savoly et al. ..... 166/293  
 4,690,589 9/1987 Owa ..... 405/263  
 4,692,065 9/1987 Suzuki et al. ..... 405/211  
 4,720,214 1/1988 Brasted et al. .

- 4,746,245 5/1988 Mork ..... 405/224  
 4,760,882 8/1988 Novak .  
 4,761,183 8/1988 Clarke .  
 4,790,954 12/1988 Burba, III et al. .  
 4,880,468 11/1989 Bowlin et al. .  
 4,897,119 1/1990 Clarke .  
 4,913,585 4/1990 Thompson et al. .  
 4,942,929 7/1990 Malachosky et al. .  
 4,991,668 2/1991 Rehm et al. .  
 5,016,711 5/1991 Cowan .  
 5,020,598 6/1991 Cowan et al. ..... 166/293  
 5,026,215 6/1991 Clarke .  
 5,058,679 10/1991 Hale et al. .  
 5,082,499 1/1992 Shen ..... 106/735  
 5,086,850 2/1992 Harris et al. .  
 5,105,885 4/1992 Bray et al. .  
 5,106,423 4/1992 Clarke .  
 5,121,795 6/1992 Ewert et al. .  
 5,123,487 6/1992 Harris et al. .  
 5,125,455 6/1992 Harris et al. .  
 5,127,473 7/1992 Harris et al. .  
 5,133,806 7/1992 Sakamoto et al. ..... 106/811  
 5,147,565 9/1992 Bour et al. ..... 252/8.551

## FOREIGN PATENT DOCUMENTS

- 85144069/24 7/1983 Japan .  
 61-48454 3/1986 Japan .  
 833704 6/1981 U.S.S.R. .

## OTHER PUBLICATIONS

- Smith, Dwight K., "Open-Hole Cement Plugs", *Cementing*, 1976, pp. 97-102.  
 "Deep Cement Mixing Experience in Japan", by G. Dennis et al, Copyright 1985 Seabed Strengthening Symposium, Denver, Colo., Jun. 4, 1985, TP 85-5.  
 "Mud Disposal: An Industry Perspective", Hanson et al, Drilling, May 1986, pp. 16-21.  
 "Waste Minimization Program Can Reduce Drilling Costs", Hall et al, Oryx Energy Co., Houston, Tex., Oil & Gas Journal, Jul. 1, 1991, pp. 43-46.  
 "Phosphoric Acids and Phosphates", Kirk-Othmer Enc. of Chemical Technology, 3rd Ed., vol. 17, p. 477.  
 "Conversion of Drilling Fluids to Cements with Blast Furnace Slag-Performance Properties and Applications for Well Cementing", SPE Paper 24575 (Oct. 4, 1992) by Cowan et al.  
 "Quantitative Interpretation of X-Ray Diffraction Patterns of Mixtures. I. Matrix-Flusing Method for Quantitative Multicomponent Analysis", by Frank H. Chung, J. Appl. Cryst. (1974) 7, pp. 519-525.

Primary Examiner—George A. Suchfield

## [57] ABSTRACT

Method for restoring drilling fluid circulation to a borehole having strata being invaded by the drilling fluid, by circulating a non-conventional cementitious slurry such as drilling fluid-blast furnace slag mixture into the strata, and allowing the mixture to solidify in situ.

12 Claims, No Drawings

## **RESTORING LOST CIRCULATION**

## BACKGROUND OF THE INVENTION

## 1. Field of the Invention

This invention relates to a method of restoring lost circulation of drilling fluid in a well.

## 2. State of the Art

Rotary drilling of a borehole is accomplished by rotating a drill string having a drill bit at its lower end. Weight is applied to the drill string while rotating to create a borehole into the earth. The borehole may pass through numerous different strata before the borehole reaches the desired depth. The drill string is usually hollow for reasons which become apparent later. Sections are added to the drill string to increase its length as the borehole is deepened.

This drilling process creates significant amounts of friction which produces heat along with fragments of the strata being penetrated. The fragments of strata must be removed from the borehole and the drill bit must be cooled to extend its usable life. Both of these necessities are accomplished by the circulation of a drilling fluid down through the drill string and up the annulus between the drill string and borehole wall to the surface. Cooling of the drill bit is accomplished by a steady flow of cool fluid from the surface and cutting fragments are carried up the annulus to the surface where they are separated from the drilling fluid.

Drilling fluids typically include water and a complicated mixture of clays, polymeric thickeners and dispersants, and weighting agents. The properties of the drilling fluid are dictated primarily by the physical nature of the geologic formation through which the borehole will be created. The hardness, fluid content, type of fluid, porosity, permeability, in-situ stresses, compressive and tensile strength, and chemical composition are all important characteristics of a geologic formation which impact the formulation of the drilling fluid.

In addition to providing cooling, lubrication and cuttings removal from the borehole, the drilling fluid also provides pressure control for the well. A hydrostatic pressure is produced by the column of drilling fluid in the borehole. The density of the drilling fluid may be varied to produce a hydrostatic pressure at specific points along the borehole which is equivalent to or slightly in excess of the pressure of the exposed geologic formations.

In some cases, the hydrostatic pressure of the drilling fluid column required to control a formation pressure in part of the borehole may exceed the tensile or compressive strength of other exposed formations. If this happens, a fracture may be initiated and propagated in the weaker strata. This causes an alteration in the drilling fluid circulation circuit. Instead of returning to the surface up the annulus, some or all of the drilling fluid will exit the borehole through the created fracture or fractures. This is commonly referred to in drilling practice as "lost circulation".

Lost circulation may be caused by created fractures due to excessive mechanical or hydrostatic pressures applied to exposed strata, natural fractures existing in the strata, or simply by high porosity and permeability within a strata. In all cases, it is important to the drilling process to restore the circulation back to the surface within the borehole. Many materials are used for this purpose and most are bridging additives which can be

added to the drilling fluid to block the leak path of the exiting fluid.

Materials such as cottonseed hulls, ground mica, graded sand, walnut or other nut hulls ground to different sizes, diatomaceous earth, gilsonite, ground coal, charcoal, cellophane flakes, and shredded paper are common materials used as lost circulation additives added to drilling fluids. These materials are simply bridging agents and do not form a high strength solid material to seal the leak path.

Portland cement mixtures are often used to provide a more permanent seal than the non-hydraulic drilling fluid additives described earlier. One of the limitations of Portland cement formulations is their susceptibility to drilling fluid contamination. Contamination of the cement slurry with drilling fluid often reduces the compressive strength of the set cement, may greatly extend the setting time of the slurry, and may affect the bonding of the cement to the formation. This is particularly true if the drilling fluid contains significant concentrations of lignosulfonate thinners, carboxylate/hydroxide polymers such as starch, hydroxyethyl cellulose, carboxymethyl cellulose, carboxymethyl hydroxyethyl cellulose, or polyalcohols.

Another limitation of Portland cement mixtures is density. As discussed supra, the cause of the lost circulation problem may be use of a heavy mud which causes fracture initiation or propagation in strata surrounding the borehole. Portland cement mixtures are relatively dense and may simply aggravate this problem. Diluting the Portland cement to reduce its density is not an acceptable solution to this problem since the dilution weakens the Portland cement (i.e. Portland cement is very sensitive to its water/cement ratio).

Yet another limitation of Portland cement is the adverse effect of brine which causes severe strength loss.

Accordingly, the present invention is directed to overcoming the above noted problems in the art, and in particular to problems experienced with effective sealing of strata in oil and gas wells which are causing lost circulation.

## SUMMARY OF THE INVENTION

5 It is the primary purpose of the present invention to provide methods for restoring lost drilling fluid circulation of a borehole of a well.

The purpose of the invention is achieved through a method for restoring drilling fluid circulation to a bore-hole of a well having surrounding strata being invaded by the drilling fluid which is thereby escaping the bore-hole, comprising:

## preparing a cementitious slurry comprising:

(a) a cementitious component selected from blast furnace slag and a proton acceptor metal compound and

(b) an activator wherein, when said cementitious component is said blast furnace slag, said activator is optionally an alkaline agent, and when said cementitious component is said metal compound, said activator

0 tious component is said metal compound, said activator is a phosphorus acid or one of a polymer component of the formula:



wherein A is

-continued



or a mixture of



and wherein R is H or a 1-10 carbon atom alkyl radical and the ratio of m to n is within the range of 0:1 to 100:1, and

(c) a water source selected from water, brine, seawater, water base drilling fluid, and water emulsion drilling fluid;

displacing the cementitious slurry into the strata which the first said drilling fluid is invading, the cementitious slurry being in direct contact, during and after placement, with the drilling fluid in the borehole; and

allowing the cementitious slurry to solidify in situ to seal the strata from the wellbore.

The cementitious slurry may be a blend of one or more cementitious components and one or more activators. Further, the cementitious component can be a proton acceptor metal compound and the activator may be a polymer compound and phosphorous acid. The cementitious component may also be comprised of blast furnace slag and employ an activator that comprises one or more alkaline gents and a polymer. Alternatively, granulated water-quenched blast furnace slag may be employed in the cementitious slurry without incorporating an activator.

Other purposes, distinction over the art, advantages and features of the invention will be apparent to one skilled in the art upon review of the following.

#### DESCRIPTION OF PREFERRED EMBODIMENTS

The following preferred embodiments of the invention explain the principles of the invention.

The present invention provides a unique method devised to provide sealing of strata, commonly known as "thief zones", surrounding boreholes and causing lost circulation for vertical, deviated, and horizontal wells. The invention offers the permanent sealing quality associated with Portland cements without the sensitivity to drilling fluid contamination. The present invention uses a non-conventional cementitious slurry which will flow into the fractures, or porosity of the strata and form a plus. The non-conventional cement, unlike Portland cement, is not adversely affected by drilling fluid or by brine. In fact, brine significantly strengthens the blast furnace slag embodiment of the non-conventional cements, as compared to fresh water.

The density of the non-conventional cementitious slurry may be varied to meet the pressure conditions within the borehole to prevent the creation of or additional propagation of fractures in the strata. A slightly

higher density of the slurry would increase the likelihood that the fluid would invade the formation zone to which circulation is lost. A slightly lower density would reduce the likelihood of fracture initiation or propagation. Density of the slurry may be readily reduced by dilution (e.g. with water) since the non-conventional cementitious slurry is relatively unaffected by such dilution. As discussed supra, Portland cement is very sensitive to its water/cement ratio and dilution can significantly reduce the strength of Portland cement.

On the other hand, a comparatively heavy mud may have been necessary to keep out undesirable fluids from various formations through which the well bore passes. In this situation it may be necessary to use a comparatively dense cementitious slurry. This is not a problem with the slag cementitious slurry because its density is readily varied without adverse effects.

The detection of lost circulation will generally occur in two ways, i.e. either circulation of the drilling fluid will stop, indicating total loss of the drilling fluid somewhere in the borehole, or a reduced rate of circulation of the drilling fluid through the borehole will be noted, i.e. more drilling fluid is being put in than is being taken out. The type or extent of lost circulation will dictate, to some degree the response in correcting the lost circulation, e.g., total loss of circulation or substantial loss of circulation will require the injection of more cementitious slurry. Accordingly, the loss of drilling fluid circulation while drilling is restored by setting the cement plug across the thief zone and then drilling back through the plug in accordance with practices known to the art. Although much of the slurry itself may be lost to the thief zone, it will harden and consolidate the formation. A plug can also be set on top of the thief zone to protect it from fracturing under the hydrostatic pressure that might be encountered when setting and cementing the casing.

Drilling of the borehole is preferably conducted with a universal fluid which is a drilling fluid containing the non-conventional cementitious slurry. This results in a settable filter cake being deposited on the borehole wall. The settable filter cake decreases the chances of a thief zone gaining entry to the borehole and tends to restrict the size of the entry of the thief zone to the borehole. In addition, the settable filter cake furnishes an excellent means for bonding the lost circulation plug to the borehole in order to effectively seal the thief zone.

Cementing of the well is preferably conducted by adding the non-conventional cementitious slurry to the universal fluid. This results in a cement which readily bonds to the drilled-through lost circulation plug and to the settable filter cake. Of course it is manifest that drilling and cementing may be conducted with conventional fluids known to the art which work well with the lost circulation plug of this invention.

#### DETAILED DESCRIPTION OF THE INVENTION

In this description the term 'cementitious material' means either an hydraulic material which on contact with water and/or activators hardens or sets into a solidified composition or a component which, on contact with a reactive second component, sets or hardens into a solidified composition. Thus, broadly it can be viewed as a material which can chemically combine to form a cement. A slurry of the cementitious material and the component or components which

cause it to harden is referred to herein as a cementitious slurry. The term 'pipe' means a casing or liner.

### DRILLING FLUIDS

The initial drilling fluid or mud can be either a conventional drilling fluid, i.e., one not containing a cementitious material, or it can be one already containing a cementitious material in a relatively small amount. The drilling fluid can be either a water-based fluid or an oil-based fluid. The term 'water-based fluid' is intended to encompass both fresh water muds, salt water containing muds, whether made from seawater or brine, and other muds having water as the continuous phase including oil-in-water emulsions. In any event drilling fluid will always contain at least one additive such as 10 viscosifiers, thinners, dissolved salts, solids from the drilled formations, solid weighting agents to increase the fluid density, formation stabilizers to inhibit deleterious interaction between the drilling fluid and geologic formations, and additives to improve the lubricity of the 20 drilling fluid.

It is generally preferred that the water-based drilling fluids use water containing dissolved salts, particularly sodium chloride. In these instances, 0 to up to saturation, preferably 0.5 to 20, more preferably 0.2 to 5 wt % sodium chloride may be used. One suitable source is to use seawater or a brine solution simulating seawater. Particularly in the embodiment using slag, the strength of the resulting cement is actually enhanced which is contrary to what would be expected in view of the 30 intolerance of Portland cement to brine. Various salts, preferably organic salts, are suitable for use in the drilling fluid used in this invention in addition to, or instead of NaCl, including, but not limited to, NaBr, KCl, CaCl<sub>2</sub>, NaNO<sub>2</sub>, NaC<sub>2</sub>H<sub>3</sub>O<sub>2</sub>, KC<sub>2</sub>H<sub>4</sub>O<sub>2</sub>, NaCHO<sub>2</sub> and 35 KCHO<sub>2</sub> among which sodium chloride is preferred, as noted above. The term 'oil-based fluids' is meant to cover fluids having oil as the continuous phase, including low water content oil-base mud and invert oil-emulsion mud.

A typical mud formulation to which cementitious material may be added to form drilling fluid is as follows: 10-20 wt % salt, 8-10 lbs/bbl bentonite, 4-6 lbs/bbl carboxymethyl starch (fluid loss preventor), sold under the trade name "BIOLOSE" by Milpark, 0.5-1 lbs/bbl partially hydrolyzed polyacrylamide (PHPA) which is a shale stabilizer, sold under the trade name "NEWDRIL" by Milpark, 1-1.25 lbs/bbl CMC sold under the trade name "MILPAC" by Milpark, 30-70 lbs/bbl drill solids, and 0-500 lbs/bbl barite.

The term 'universal fluid' is used herein to designate those compositions containing cementitious material, which compositions are suitable for use as a drilling fluid, and which compositions thereafter, for the purpose of practicing this invention, have additional cementitious material and/or activators such as accelerators (or reactive second components) added to give a cementitious slurry.

Thus, with the universal fluid embodiment of this invention, the purpose of one aspect of the invention is achieved through a method for drilling and cementing a well comprising preparing a universal fluid by mixing a drilling fluid and a cementitious material; drilling a borehole with the universal fluid and laying down a settable filter cake on the walls of the borehole during 60 drilling of the well; diluting the drilling fluid; adding additional cementitious material and/or accelerators (or reactive second components) and introducing the thus-

formed cementitious slurry into the wellbore and into an annulus between the wellbore and a casing where it hardens and sets up forming a good bond with the filter cake which filter cake, with time, actually hardens itself because of the presence of cementitious material therein. This hardening is facilitated by any accelerators which may be present in the cementitious slurry and which migrate by diffusion and/or filtration into the filter cake.

### NON-CONVENTIONAL CEMENTS

The cementitious component can be any one or more of: conventional hydraulic cement, natural or artificial pozzolan, or the metal compound used to produce an ionomer or to produce a phosphorus salt. The preferred cementitious material is one selected from the group consisting of blast furnace slag, a metal compound which is a proton acceptor component used to produce the ionomer and a metal compound which is a proton acceptor component used to produce the phosphorus salt. By 'blast furnace slag' is meant the hydraulic refuse from the melting of metals or reduction of ores in a furnace as disclosed in Hale and Cowan, U.S. Pat. No. 5,058,679 (Oct. 22, 1991), the disclosure of which is hereby incorporated by reference. By 'phosphorus salt' is meant a phosphonate, a phosphate or a polyphosphate as is described in detail hereinafter.

The preferred blast furnace slag used in this invention is a high glass content slag produced by quickly quenching a molten stream of slag at a temperature of between 1400° C. and 1600° C. through intimate contact with large volumes of water. Quenching converts the stream into a material in a glassy state having hydraulic properties. At this stage it is generally a granular material that can be easily ground to the desired degree of fineness. Silicon dioxides, aluminum oxides, iron oxides, calcium oxide, magnesium oxide, sodium oxide, potassium oxide, and sulphur are some of the chemical components in slags. Preferably, the blast furnace slag used in this 40 invention has a particle size such that it exhibits a Blaine specific surface area between 500 cm<sup>2</sup>/g and 15,000 cm<sup>2</sup>/g and more preferably, between 3,000 cm<sup>2</sup>/g and 15,000 cm<sup>2</sup>/g, even more preferably, between 4,000 cm<sup>2</sup>/g and 9,000 cm<sup>2</sup>/g, most preferably between 4,000 cm<sup>2</sup>/g and 8,500 cm<sup>2</sup>/g. An available blast furnace slag which fulfills these requirements is marketed under the trade name "NEWCEM" by the Blue Circle Cement Company. This slag is obtained from the Bethlehem Steel Corporation blast furnace at Sparrows Point, Md.

50 A usual blast furnace slag composition range in weight percent is: SiO<sub>2</sub>, 30-40; Al<sub>2</sub>O<sub>3</sub>, 8-18; CaO, 35-50; MgO, 0-15; iron oxides, 0-1; S, 0-2 and manganese oxides, 0-2. A typical specific example is: SiO<sub>2</sub>, 36.4; Al<sub>2</sub>O<sub>3</sub>, 16.0; CaO, 43.3; MgO, 3.5; iron oxides, 0.3; S, 0.5; and MnO<sub>2</sub>O<sub>3</sub><0.1.

Blast furnace slag having relatively small particle size is frequently desirable because of the greater strength it imparts in many instances to a final cement. Characterized in terms of particle size the term "fine" can be used 60 to describe particles in the range of 4,000 to 7,000 cm<sup>2</sup>/g Blaine specific surface area. Corresponding to 16 to 31 microns in size; "microfine" can be used to describe those particles in the 7,000 to 10,000 cm<sup>2</sup>/g Blaine specific surface area range that correspond to particles of 5.5-16 microns in size and "ultrafine" can be used to describe particles over 10,000 cm<sup>2</sup>/g Blaine specific surface area that correspond to particles 5.5 microns and smaller in size.

However, it is very time consuming to grind blast furnace slag to these particle sizes. It is not possible to grind blast furnace slag in a manner where particles are entirely once size. Thus, any grinding operation will give a polydispersed particle size distribution. A plot of particle size versus percent of particles having that size would thus give a curve showing the particle size distribution.

In accordance with a preferred embodiment of this invention a blast furnace slag having a polydispersed particle size distribution exhibiting at least two nodes on a plot of particle size versus percent of particles in that size is utilized. It has been found that if only a portion of the particles are in the ultrafine category, the remaining, indeed the majority, of the slag can be ground more coarsely and still give essentially the same result as is obtained from the more expensive grinding of all of the blast furnace slag to an ultrafine state. Thus, a grinding process which will give at least 5% of its particles falling within a size range of 1.9 to 5.5 microns offers a particular advantage in economy and effectiveness. More preferably, 6 to 25 wt % would fall within the 1.9 to 5.5 micron range. The most straightforward way of obtaining such a composition is simply to grind a minor portion of the blast furnace slag to an ultrafine condition and mix the resulting powder with slag ground under less severe conditions. Even with the less severe conditions there would be some particles within the fine, microfine or ultrafine range. Thus, only a minority, i.e., as little as 4 wt % of the slag, would need to be ground to the ultrafine particle size. Generally, 5 to 20 wt %, more preferably 5 to 8 wt % can be ground to the ultrafine particle size and the remainder ground in a normal way thus giving particles generally in a size range of greater than 11 microns, the majority being in the 11 to 31 micron range.

By ionomer is meant organometal compositions having a metal attached to or interlocking (crosslinking) a polymer chain. Suitable polymer components of such ionomers can be represented by the formula



wherein A is



or a mixture of



and wherein R is H or a 1-10 carbon atom alkyl radical. The ratio of m to n is generally within the range of 0:1 to 100:1, preferably 0.1:1 to 10:1.

The polymers generally have a ratio of functional groups to polymer chain carbons within the range of 1:2 to 1:10, preferably about 1:3. Thus, if m and n are 1, R is H and A is carboxylate, there would be a ratio of carboxylic carbons (1) to polymer chain carbons (4) of 1:4. The polymer can also be a polycarboxylic acid polymer. One such polymer is that made from partially hydrolyzed polyacrylamide. The hydrolysis can vary from 1% up to 100% and preferably from 10% to 50%, most preferably from 25% to 40%. The molecular weight of the polymers can vary widely so long as the polymers are either water-soluble or water-dispersible. The weight average molecular weights can range from 1000 to 1,000,000 but preferably will be in the range of 1,000 to 250,000, most preferably 10,000 to 100,000. Carboxylate polymer with a low ratio of COOH:C within the range of 1:3 to 2:5 are preferred. Especially preferred is a carboxylic acid polymer having a ratio of carboxylic carbons to polymer chain carbons (including carbons of pendant chains) of about 1:3 and a molecular weight within the range of 10,000 to 100,000. Partially hydrolyzed polyacrylamide polymers in the range of 5,000-15,000,000 molecular weight are suitable. The copolymers will generally have from 2-99, preferably 5-80, more preferably 10-60 mole percent acid-containing units.

The poly(carboxylic acid) component can be any water soluble or water dispersible carboxylic acid polymer which will form ionomers. Ionomer forming polymers are well known in the art. Suitable polymers include poly(acrylic acid) poly(methacrylic acid), poly(ethylacrylic acid), poly(fumaric acid), poly(maleic acid), poly(itaconic acid) and copolymers such as ethylene/acrylic acid copolymer and ethylene/methacrylic acid copolymer. The copolymers are generally random copolymers. An example of phosphonic acid polymers is poly(vinyl phosphonic acid) which is made from vinyl phosphonic acid,



Suitable copolymers containing vinyl phosphonic acid include vinyl phosphonic acid/acrylic acid copolymer as well as copolymers with other unsaturated monomers, with or without a functional group.

In some instances, it is preferred to use water dispersible, as opposed to water soluble, polymers. Ideally, in such instances the melting point of the polymer should be higher than the placement temperature (circulating temperature) in the wellbore during the "cementing" operation and lower than the maximum, static temperature of the surrounding formations. It is desirable for the polymer to melt and react after placement as the temperature in the wellbore increases from the circulating temperature to the static temperature of the surrounding formations.

The ionomers suitable for use in this invention are the water-insoluble reaction product of a proton acceptor metal compound which serves as the cementitious component and a carboxylic, sulfonic, or phosphonic acid polymer component. The metal compound generally is

a metal oxide such as CaO, MgO or ZnO. The preferred metal oxides are magnesium oxide and zinc oxide, and most preferably, magnesium oxide. The applicable metal oxides are generally fired at temperatures above 1,000° F. for several hours to reduce chemical activity prior to grinding to final particle size for use in reacting with the acid component.

In instances where it is desired that the metal compound component add weight to the drilling fluid, the metal compound is preferably a water-insoluble metal compound with a specific gravity of at least 3.0, preferably 3.5. By 'insoluble' is meant that less than 0.01 parts by weight dissolve in 100 parts by weight of cold (room temperature) water.

The particle size of the metal compound component can vary widely. Generally, it will be within the range such that the powder exhibits a surface area within the range of 500  $\text{cm}^2/\text{g}$  to 30,000  $\text{cm}^2/\text{g}$ , preferably 1,500  $\text{cm}^2/\text{g}$  to 25,000  $\text{cm}^2/\text{g}$ , most preferably 2,000  $\text{cm}^2/\text{g}$  to 20,000  $\text{cm}^2/\text{g}$ .

The amount of polymer utilized will vary widely depending upon the carboxylic acid content of the polymer; broadly, 10 to 200, preferably 10 to 100, most preferably 10 to 80 wt %, based on the weight of metal compound, can be present. With the polymers having a low ratio of m to n, a smaller amount is required because of the higher functional group content of the polymer. Conversely, with the high ratio of m to n, an amount of polymer toward the higher end of the ranges is preferred. Polymers with ester groups can be used to delay or retard the setting of the cement.

Phosphates and phosphonates, referred to herein as phosphorus salts, used in accordance with this invention also are produced from a two-component composition, the first component of which is a metal compound identical in scope to that used in the ionomers as described hereinabove so long as the resulting phosphorus salt is insoluble in water. Most preferred are CaO, MgO and ZnO.

The second component is a phosphonic or phosphoric acid, preferably a polyphosphoric acid. The term 'phosphoric acid' is meant to encompass both linear and cyclic polyphosphoric acids. These second component acids are referred to herein as phosphorus acids. Linear phosphoric acids can be depicted by the general formula  $H_{n+2}P_nO_{3n+1}$  where n is 1 to 100, preferably 2 to 50, more preferably, 2 to 20. Examples include di-(pyro)phosphoric acid, tri-(tripoly)phosphoric acid, tetra-phosphoric acid and higher molecular weight polyphosphoric acids as well as phosphoric acid. Mixtures of acids, including those traditionally referred to as meta phosphoric acid, are particularly suitable for use in this invention.

The formation of one phosphate cement using a metal oxide as the metal compound can be depicted as follows:



where:

X is usually 4; and

MO=metal oxide which is amphoteric or is a proton acceptor.

The phosphorus acid component is used in a stoichiometric amount or less since an excess of acid should generally be avoided. From 1 to 10 or even to 50 mole percent less than a stoichiometric amount is suitable. Generally, a stoichiometric amount will be between 10 and 100 wt % based on the weight of the metal compound. Boric acid, borate salts, and aluminates such as sodium aluminate can be used, in an amount of 1-100% by weight based on the weight of the phosphorus acid, to delay or retard the setting of the phosphate cement.

With the ionomers, and the phosphorus salts when made with a polyvalent metal compound, a crosslinked network structure exists as a result of the addition of the second component, thus giving a very strong solid cement.

Because of the mass provided by the metal compound component of the ionomer or the polyphosphorus salt, these cementitious materials are generally actually heavier than most slag or Portland cement materials. In the embodiments using these cementitious materials this high density provides significant advantages in certain utilities. For one thing, a smaller amount of the material can be used and still achieve a final mud and ultimately a cement of a desired density. Secondly, because of the high density, it is possible to operate without weighting agents such as barium sulfate or barite. They offer a further advantage in that they do not set up until the second component is added.

The metal compound of the ionomer or phosphorus salt can be used as the sole cementitious material or can be used in admixture with siliceous hydraulic materials such as the blast furnace slag or Portland cement. In one embodiment an hydraulic component such as slag can be used to give the metal ion component of the ionomer or phosphate to give, in effect, a mixture formed in situ.

Preferably, when the ionomer or phosphorus salt is utilized, the metal compound is added first and thereafter at such time as it is desired for the cement to be activated to set, the other component is added. In the case of the universal fluids, a portion of the total metal compound can be added to the drilling fluid, the remainder being added after dilution when the cementitious slurry is being formed.

The sequence for the universal fluid embodiment of this invention is to prepare the drilling fluid containing a portion of the total slag or metal compound to be utilized, carry out the drilling operation, dilute the fluid, 50 add the remainder of the slag or metal compound, and thereafter add the activator or acid components and utilize the cement for its intended purpose such as cementing a casing.

In accordance with the invention that utilizes universal fluid, the fluid itself becomes a part of the final cement and thus, this portion of the drilling fluid does not need to be disposed of.

In all embodiments of the invention, additional cement can be made and used, in accordance with this invention, for remedial cementing.

The ionomer embodiments of this invention are of particular value for filling and sealing the annulus between a borehole wall and a casing, or between casings, particularly where some degree of ductility and/or tensile strength is desired. The ionomer has good adhesive properties to the borehole wall and casing and has greater elasticity than is obtained with siliceous hydraulic materials such as Portland cement. Thus, such ce-

ments are resistant to cracking under conditions of cyclic loading as are frequently encountered in a wellbore. For similar reasons the ionomer embodiment of the invention is beneficial in cementing liners and tieback casing strings which may otherwise leak due to changes in pressure and temperature in the well during production operations. Another area where the ductility of the ionomer cement is of special value is in slim hole wells where the annulus is smaller. Still yet another area where this ductility is important is in extended reach drilling. The term 'extended reach' is intended to cover horizontal drilling and any other well drilling operations which are off-vertical a sufficient amount to cause the casing to be displaced by gravity toward one side of the borehole.

As noted hereinabove the initial drilling fluid can be either a conventional drilling fluid or it can be a universal fluid which already has cementitious material therein.

### DILUTION

In all embodiments, the amount of dilution can vary widely depending on the desired application. Generally, the fluid will be diluted with from 5 to 200 by volume, preferably 5 to 100% by volume, more preferably 5 to 50% by volume of liquid (water in the case of a water-based fluid) based on the volume of initial drilling fluid. In one particularly preferred embodiment, the dilution is such that on addition of the cementitious component (or in the case of the universal fluid addition of the remaining cementitious component) the final density will be within the range of 30% less to 70% more than the original density, preferably within the range of 15% less to 50% more, preferably, essentially the same, i.e., varying by no more than  $\pm 5$  wt %. This is particularly valuable in an operation where there is a narrow pressure window between the pressure needed to prevent blowout and the pressure which would rupture or fracture the formation through which drilling has taken place.

The dilution fluid can be the same or different from that used to make the drilling fluid in the first place. In the case of brine-containing fluids the dilution fluid will generally be brine also. This is of particular benefit in offshore drilling operations where fresh water is not readily available but brine is since seawater is a desirable brine.

Thus, as noted above, a significant improvement in the operating procedure is provided in accordance with this invention. This is because the density of the drilling fluid is frequently tailored to the characteristics of the formation through which the wellbore is being drilled. Thus, the density is chosen in the first place to be sufficient to avoid inflow into the wellbore because of formation pressure but is further chosen to be insufficient to rupture or fracture the borehole wall and force the fluid out into the formation. By utilizing the dilution and thereafter addition of the cementitious component (or in the case of universal fluid, the remainder of the 60 cementitious component) the cementitious slurry can likewise have a density tailored to the particular operation. In addition, this avoids undue thickening of the drilling fluid as would occur, particularly with some hydraulic components, without the dilution and thus the rheological properties of the cementitious slurry and the drilling fluid can both be tailored for optimum performance.

The invention (dilution of a drilling fluid and thereafter adding cementitious material to produce a cementitious slurry) offers special advantages with certain cementitious components in addition to the general benefits such as reduced equipment needs. With Portland cement it reduces the extraordinary viscosity increase that adding such an hydraulic material to a drilling fluid would give. With slag, organometals and polyphosphates there is the advantage that the cementitious component has a drilling fluid function. With the ionomers and polyphosphates there is the further general advantage that unlimited time can elapse between the drilling and cementing operations with no loss of properties of either because these materials do not begin to set until the second component is added.

The dilution can be carried out in either of two ways. First, a vessel containing drilling fluid can simply be isolated and the desired amount of water or other diluent added thereto. In a preferred embodiment, however, the drilling fluid is passed to a mixing zone as a flowing stream and the dilution fluid added "on the fly" to the flowing stream. Thereafter the additional blast furnace slag is added. This avoids highly viscous cementitious slurry compositions and allows all of the pumping to be done with piping and pumps associated with the well rig without the need for pumps designed for pumping cement. This is of particular value in the areas to which this invention is of special utility, offshore drilling rigs where the transportation of additional pumping equipment is particularly inconvenient. Thus, it is possible to tailor the final density of the cementitious slurry, if desired, to a value within the range of 30% less to 70% more than the original density of the drilling fluid, preferably within the range of 15% less to 50% more, most preferably essentially the same, i.e., varying by no more than  $\pm 5$  weight percent.

Mixed metal hydroxides can be used in the drilling fluid to impart thixotropic properties. The mixed metal hydroxides provide better solids suspension. This, in combination with the settable filter cake provided in the technique of this invention, greatly enhances the cementing in a restricted annulus. The mixed metal hydroxides are particularly effective in muds containing clay such as sodium bentonite. Preferred systems thickened in this way contain from 1-20 lbs/bbl of clay such as bentonite, preferably 2 to 15 lbs/bbl, most preferably 7 to 12 lbs/bbl. The mixed metal hydroxides are generally present in an amount within the range of 0.1 to 2 lbs/bbl of total drilling fluid, preferably 0.1 to 1.5 lbs/bbl, most preferably 0.7 to 1.2 lbs/bbl. Mixed metal hydroxides are known in the art and are trivalent metal hydroxide-containing compositions such as  $MgAl(OH)_{4.7}Cl_{0.3}$ . They conform essentially to the formula



where

M represents the number of Li ions present; the said amount being in the range of zero to about 1;

D represents divalent metals ions; with d representing the amount of D ions in the range of zero to about 4;

T represents trivalent metal ions;

A' represents monovalent or polyvalent anions of valence  $-n$ , other than  $OH^-$ , with a being the amount of A' anions; and

where  $(m+2d+3+na)$  is equal to or greater than 3. A more detailed description can be found in Burba, U.S.

Pat. No. 4,664,843 (May 12, 1987). The mixed metal hydroxides in the drilling fluid, in combination with blast furnace slag, tend to set to a cement having considerable strength in a comparatively short time, i.e., about one-half hour at temperatures as low as 100° F. This can be a major asset in some applications. In such instances, a thinner such as a lignosulfate is preferably added before adding slag. However, one of the advantages of this invention is that it reduces or eliminates the need for additives to control free water or solids suspension. The activator or activators can be added either with any other ingredients that are added before the additional blast furnace slag, with the additional blast furnace slag, or after the addition of the additional blast furnace slag.

In some instances, it may be desirable to use a material which functions as a retarder along with the activator because of the need for other effects brought about by the retarder. For instance, a chromium lignosulfonate may be used as a thinner along with the activator even though it also functions as a retarder.

Other suitable thinners include chrome-free lignosulfonate, lignite, sulfonated lignite, sulfonated styrene maleic-anhydride, sulfomethylated humic acid, naphthalene sulfonate, a blend of polyacrylate and polymethacrylate, an acrylamideacrylic acid copolymer, a phenol sulfonate, a naphthalene sulfonate, dodecylbenzene sulfonate, and mixtures thereof.

In one embodiment the drilling fluid consists essentially of slag and seawater and is pumped exclusively using the piping and pumps associated with the drilling rig without the need for any pumps designed for pumping cement.

In the case of hydraulic materials, particularly the more preferred hydraulic material, blast furnace slag, the amount of hydraulic material present in the universal fluid is generally within the range of 1 to 100 lbs/bbl of final drilling fluid, preferably 10 to 80 lbs/bbl, most preferably 20 to 50 lbs/bbl. In the case of the organometals (ionomers) or phosphorus salts the amount of metal compound initially present in universal fluid can also vary widely. Generally, 1 to 500 lbs/bbl, preferably 50 to 300 lbs/bbl, most preferably 100 to 250 lbs/bbl of the metal compound are used.

The total amount of cementitious material in the cementitious slurry will typically range from about 20 lbs/bbl to about 600 lbs/bbl, preferably 100 lbs/bbl to 500 lbs/bbl, most preferably 150 lbs/bbl to 350 lbs/bbl. This can be adjusted to give the desired density as noted hereinabove.

Reference herein to additives encompasses both the specialized additives necessary for this invention such as the carboxylic acid polymer in the case of the ionomer or the polyphosphoric acid in the case of the polyphosphate as well as conventional additives.

#### CONVENTIONAL DRILLING FLUID ADDITIVES

Suitable fluid loss additives found in drilling fluids include bentonite clay, carboxymethylated starches, starches, carboxymethyl cellulose, synthetic resins such as "POLYDRILL" by SKW Chemicals, sulfonated lignite, lignites, lignin, or tannin compounds. Weight materials include barite, calcium carbonate, hematite and MgO, for example. Shale stabilizers that are used in drilling fluids include hydrolyzed polyacrylonitrile, partially hydrolyzed polyacrylamide, salts including NaCl, KCl, sodium or potassium formate, sodium or

potassium acetate, polyethers and polycyclic and/or polyalcohols. Viscosifying additives can be used such as biopolymers, starches, attapulgite and sepiolite. Additives are also used to reduce torque. Suitable thinners such as chrome and chrome free lignosulfonates, sulfonated styrene maleic-anhydride and polyacrylate may also be used depending upon the mud type and mud weight. Lubricating additives include nonionic detergents and oil (diesel, mineral oil, vegetable oil, synthetic oil), for instance. Alkalinity control can be obtained with KOH, NaOH or CaO, for instance. In addition, other additives such as corrosion inhibitors, nut hulls etc. may be found in a typical drilling fluid. Of course, drill solids including such minerals as quartz and clay minerals (smectite, illite, chlorite, kaolinite, etc.) may be found in a typical mud.

It is particularly desirable in accordance with a further embodiment of this invention to utilize silica to increase the temperature resistance of the final cement. The use of blast furnace slag as the hydraulic component, in itself, allows greater latitude in the temperature which can be tolerated, because the blast furnace slag is inherently less thermally sensitive than other known hydraulic components such as Portland cement and thus can be hardened over a wider range of temperatures without resort to additives. This is of particular advantage where there is a substantial temperature gradient from the top to the bottom of a borehole section to be cemented. However, with the addition of silica, further temperature resistance may be imparted to the cement after it is set. Thus, with blast furnace slag and silica a temperature resistant cement is possible and with other cementitious components the temperature range can be extended through the used silica. Suitable silicas include crystalline silicas such as alpha quartz.

#### UNIVERSAL FLUIDS

In another embodiment of this invention, most or all of the components of the drilling fluid are chosen such that they have a function in the cementitious material also. The following Table illustrates the uniqueness of such formulations.

TABLE A

| Additive                          | Function               |                              |                           |                            |
|-----------------------------------|------------------------|------------------------------|---------------------------|----------------------------|
|                                   | Drilling Fluid         |                              | Cementitious Slurry       |                            |
| Primary                           | Secondary              | Primary                      | Secondary                 |                            |
| Synthetic polymer <sup>1</sup>    | Fluid loss control     |                              | Fluid loss control        | Retarder                   |
|                                   | Fluid loss control     | Viscosity                    | Fluid loss control        | Retarder                   |
|                                   |                        | Viscosity                    | Viscosity                 | Retarder                   |
| Starch <sup>2</sup>               |                        |                              |                           |                            |
|                                   | Viscosity              | Shale stabilizer             | Accelerator               | —                          |
| Biopolymer <sup>3</sup>           |                        |                              |                           |                            |
|                                   | Viscosity              | Deflocculant                 | Retarder                  | Deflocculant               |
| Silicate                          |                        |                              |                           |                            |
|                                   | Density                | —                            | Density concentration     | Solids                     |
| Carbohydrate polymer <sup>4</sup> | Deflocculant           | —                            | Fluid loss control        | Solids concentr.           |
|                                   |                        | Density                      | Solids concentration      | —                          |
| Barite <sup>5</sup>               |                        |                              |                           |                            |
|                                   | Bentonite <sup>6</sup> | Fluid loss control           | —                         |                            |
| Bentonite <sup>6</sup>            | —                      | —                            | —                         |                            |
|                                   |                        |                              |                           |                            |
| Clay/Quartz dust <sup>7</sup>     |                        |                              |                           |                            |
|                                   | Slag <sup>8</sup>      | Cuttings stabilizer          | —                         | Cementitious concentration |
| Slag <sup>8</sup>                 |                        | Cuttings/Wellbore stabilizer | Alkalinity                | Solids                     |
|                                   |                        | Shale stabilizer             | Accelerator concentration | Solids                     |
| Lime <sup>9</sup>                 |                        |                              |                           |                            |
|                                   | PECP <sup>10</sup>     | Fluid loss                   | Retarder                  | Rheological Control        |
|                                   |                        |                              |                           |                            |

TABLE A-continued

| Additive | Function         |         |                     |   |
|----------|------------------|---------|---------------------|---|
|          | Drilling Fluid   |         | Cementitious Slurry |   |
| Primary  | Secondary        | Primary | Secondary           |   |
| NaCl     | Shale stabilizer | —       | —                   | — |

<sup>1</sup>Polydrill, A synthetic polymer manufactured by SKW Chemicals Inc. under trade name Polydrill, for instance.

<sup>2</sup>Starch made by Milpark Inc. under the trade name "PERMALOSE", for instance.

<sup>3</sup>A biopolymer made by Kelco Oil Field Group, Inc., under the trade name "BIO-ZAN" for instance.

<sup>4</sup>Water-soluble carbohydrate polymer manufactured by Grain Processing Co. under trade name "MOR-REX".

<sup>5</sup>Barite is  $\text{BaSO}_4$ , a drilling fluid weighting agent.

<sup>6</sup>Bentonite is clay or colloidal clay thickening agent.

<sup>7</sup>Clay/quartz solid dust manufactured by MilWhite Corp. under the trade name "REVDUST", for instance.

<sup>8</sup>Blast furnace slag manufactured by Blue Circle Cement Co. under the trade name "NEWCEM" is suitable.

<sup>9</sup> $\text{CaO}$

<sup>10</sup>Polycyclicpolyetherpolyol

The material in the above Table A labeled PECP is of special significance in connection with this invention. This refers to a polyhydric alcohol most preferably a polycyclicpolyetherpolyol. A general chemical composition formula representative of one class of these materials is as follows:



where  $x \geq 1$  and  $y \geq 0$ .

A more complete description of these polycyclicpolyetherpolyols is found in the Hale and Cowan patent, U.S. Pat. No. 5,058,679 (Oct. 22, 1991), referred to hereinabove, the disclosure of which is incorporated herein by reference.

Universal drilling fluids which utilize blast furnace slag can be subsequently activated to cause the drilling fluid to develop compressive strength with time.

Suitable activators include sodium silicate, sodium fluoride, sodium silicofluoride, magnesium silicofluoride, magnesium hydroxide, magnesium oxide, zinc silicofluoride, zinc oxide, zinc carbonate, titanium carbonate, sodium carbonate, potassium sulfate, potassium nitrate, potassium nitrite, potassium carbonate, sodium hydroxide, potassium hydroxide, copper sulfate, lithium hydroxide, lithium carbonate, calcium oxide, calcium sulfate, calcium nitrate, calcium nitrite, calcium hydroxide, sodium sulfate and mixtures thereof. A mixture of caustic soda (sodium hydroxide) and soda ash (sodium carbonate) is preferred because of the effectiveness and ready availability. When mixtures of alkaline agents such as caustic soda and soda ash are used the ratio can vary rather widely since each will function as an accelerator alone. Preferably, about 1 to 20 lbs/bbl of caustic soda, more preferably 2 to 6 lbs/bbl of caustic soda are used in soda, more preferably 2 to 6 lbs/bbl, preferably 2 to 20 lbs/bbl of soda ash. The references to "lbs/bbl" means pounds per barrel of final cementitious slurry.

A combination of sodium hydroxide and sodium carbonate is preferred. In addition, blast furnace slag can be added between the use of this material as a drilling fluid and its use as a cement. The additional slag can be the activator, especially if heat is imparted to the operation. Each component is an important ingredient for both the drilling fluid and the cement. The PECP is

particularly significant in combination with slag since it acts as a retarder and thus provides significant drilling fluid functions in general and specific drilling functions relative to the slag component as well as significant cement functions. PECP also reduces the friction coefficient of muds on casing and filter cake, and pullout forces required to release stuck pipe are dramatically reduced with PECP in the drilling fluid. PECP is a rheology modifier due to its tendency to adsorb onto polymers and clays.

The unique advantage of universal fluids is that wellbore stabilization, fluid-loss control, and cuttings transport can be realized essentially the same as with conventional drilling fluid systems. However, with the simple presence of activators in the subsequent cementitious slurry, the resulting mud-slag system will develop strength. Thus, for instance,

(1) drilling fluid filter cake deposited while drilling over permeable zones can be converted into an effective sealant by diffusion of activators from the mud-slag column; and

(2), whole mud that has not been removed from washed-out sections of the hole during displacement will harden with time and, therefore, provide an effective sealant and lateral support to the casing.

In areas such as slim hole drilling, the ionomer universal fluid gives the process benefit of avoiding the removal of an incompatible drilling mud and the product benefit of being resistant to deflection when set.

In the case of the universal fluids, the amount of cementitious material can vary considerably and also can vary depending upon whether the cementitious component is a siliceous material, an organometal, or a polyphosphate.

Process and apparatus used to drill and cement are well known. One example can briefly illustrate typical practice as follows. A well is drilled using a hollow drill string having a drill bit with at least one orifice communicating between the inside of the hollow drill string and the outside and located at the lower end of the drill string, thus producing a wellbore. During this drilling, a drilling fluid is circulated down the inside of the drill string and out of the orifice at the lower end thereof. When the drilling is complete, the drill string is withdrawn from the wellbore. A first section of well casing, generally having a float shoe with an upper sealing surface, is inserted into the wellbore. Additional sections of casing are generally attached sequentially to the first section and the first section is inserted further into the wellbore. In accordance with one embodiment of this invention, additional drilling fluid, containing additives necessary to form a cementitious slurry, is pumped down the casing. This may be facilitated by inserting a bottom plug into the casing string, the bottom plug having a longitudinal passage and a rupturable diaphragm at the top, so that it is forced down the casing by the cementitious slurry. Thereafter, a top or second plug can be inserted into the casing string above the column of cementitious slurry, the diaphragm of the first plug ruptured, and the slurry forced up into an annulus between the outside of the casing and the inside of the borehole where, with time, it hardens.

In accordance with another embodiment of this invention, the use of these conventional plugs for separating the cementitious slurry from the drilling fluid is generally not necessary. In this embodiment the drill string is simply removed, a casing inserted, and the

cementitious slurry circulated into the borehole and up the annulus. This can be done by direct fluid contact between the displacement fluid and the cementitious slurry thus eliminating the need for a loading collar or wiper plug.

In yet another related embodiment of this invention, universal fluid is utilized in a drilling operation and thereafter additional cementitious material and/or additives, or the second component of a two-component system, is gradually added so as to gradually transition the circulating material from a drilling fluid to a cementitious slurry.

#### FILTER CAKE SETTING

In yet another embodiment of this invention the drilling process is carried as described hereinabove with a universal fluid to produce a borehole through a plurality of strata thus laying down a filter cake. Prior to the cementing operation the activator or reactive second component is passed into contact with the filter cake, for instance by circulating the activator or reactive second component down the drill string and up the annulus between the drill string and the filter cake. This can be accomplished by circulating a separate fluid containing the activator or reactive second component or by adding an activator or reactive second component to the drilling fluid. Alternatively, the drill string is removed and the casing inserted and the activator or reactive second component circulated down the casing and up the annulus. As used herein 'down' as it relates to a drill string or casing, means in a direction toward the farthest reach of the borehole even though in rare instances the borehole can be disposed in a horizontal position. Similarly, 'up' means back toward the beginning of the borehole. Preferably, the circulation is carried out by using the drill string, this being the benefit of this embodiment of the invention whereby the filter cake can be "set" to shut off gas zones, water loss, or to shut off lost circulation in order to keep drilling without having to remove the drill string and set another string of casing. This can also be used to stabilize zones which may be easily washed-out (salt zones wherein the salt is soluble in water, for instance) or other unstable zones. After the drilling is complete the drilling fluid is then diluted, the drill string removed, and the cementing carried out as described hereinabove.

Conventional spacers may be used in the above described sequence. Also, any left over fluid having activators therein may be displaced out of the borehole by the next fluid and/or a spacer fluid and stored for subsequent use or disposal.

In this embodiment where the filter cake is "set", the activator can be any of the alkaline activators referred to hereinabove such as a mixture of sodium hydroxide and sodium carbonate when the universal fluid contains slag, or a polymer with a functional group such as a carboxy as described hereinabove wherein the universal fluid contains a metal compound proton acceptor, or the phosphoric (or polyphosphoric) or phosphonic acid component of a phosphate or phosphonate when the universal fluid contains a metal compound proton acceptor.

In another embodiment of this invention, the drilling is done using a drilling fluid containing a metal compound to lay down a filter cake which is preferably set by circulating a polymer as described to produce an ionomer or by circulating a phosphorus acid to produce a phosphate salt. Thereafter, the cementing is done with

a cementitious slurry comprising blast furnace slag and an accelerator. Also, the use of blast furnace slag as described above for the metal compound source of an ionomer or phosphate salt can be used in this embodiment as well. Thus, ionomers or phosphorus salts can be formed as filter cake followed by cementing with blast furnace slag.

Surfactants, alcohols, or blends thereof may be used in the drilling fluids of this invention to improve bonding.

#### BONDING SURFACTANTS

The surfactants may be anionic, amphoteric, cationic, nonionic or blends thereof, e.g., nonionics with anionic or cationic surfactants.

The following surfactants, classes of surfactants, and mixtures of surfactants are particularly useful in the present invention:

##### 1. Alkanol amides (nonionic):



where R = a carbon chain (alkyl group) of 8-20 carbons (usually 10-18); H<sub>1</sub> and/or H<sub>2</sub> may be replaced by an alkanol such as ethanol or isopropanol. One or both of the H's may be replaced.

Examples: lauric monoisopropanol amide, lauric diethanol amide, coconut diethanol amide. ALKAMIDE 2106® by Alkari Chemicals, Ltd. is a coconut diethanol amide suitable for this application.

##### 2. Ethoxylated alkyl aryl sulfonate:

Examples: nonyl phenol sulfonate with 8 moles ethylene oxide, and N-decyl benzene sulfonate with 6 moles ethylene oxide.

##### 3. Amine oxides (nonionic):



where R = alkyl carbon chains from 1 to 20 carbons, usually one chain is 10 to 18 carbons. Alkyl groups can have hydroxyl or amido functional groups in their chain.

Examples: bis(2-hydroxyethyl) coco amine oxide, bis(2-hydroxyethyl) laurel amine oxide, laurel dimethyl amine oxide, coco amidopropyl dimethyl amine oxide, cetyl dimethyl amine oxide, myristyl dimethyl amine oxide.

##### 4. Betaines and Betaine Derivatives



where R<sub>1</sub> = alkyl chain length between 3 and 20 carbons, R<sub>2</sub> = alkyl chain length between 1 and 4 carbons. Amide functional groups may be incorporated into the R<sub>1</sub> alkyl chain.

Examples: coco amido propyl betaine (R<sub>1</sub> = propyl group 3 carbons), laurel betaine (R<sub>1</sub> = laurel group of 12

carbons, no R<sub>2</sub>), coco betaine (R<sub>1</sub>=coco group of 12-14 carbons, no R<sub>2</sub>), oleyl betaine (R<sub>1</sub>-oleyl group of 18 carbons, no R<sub>2</sub>), myristic betaine (R<sub>1</sub>=myristyl group of 14 carbons, no R<sub>2</sub>), oleamido propyl betaine, isostearamido propyl betaine, laurel sulfobetaine.

5. Ethoxylated Alcohols (nonionic):

Ethoxylated simple alcohols with linear or branched chains having between 8 and 20 carbons with 3 to 20 mole of ethylene oxide groups; 6-14 moles of ethylene oxide are typical.

Examples: C<sub>9</sub>-C<sub>11</sub> linear alcohol with 8 moles ethylene oxide, C<sub>14</sub>-C<sub>15</sub> linear alcohol with 13 moles ethylene oxide, C<sub>12</sub>-C<sub>15</sub> linear alcohol with 9 moles ethylene oxide.

6. Sulfates and Sulfonates of Ethoxylated Alcohols 15 (anionic):

The same ranges apply as in No. 5 supra except ethylene oxide moles may vary between 2 and 14.

Examples: C<sub>12</sub>-C<sub>13</sub> linear alcohol sulfate or sulfonate with 3 moles ethylene oxide, C<sub>12</sub>-C<sub>15</sub> linear alcohol 20 sulfate or sulfonate with 3 moles ethylene oxide.

7. Ethoxylated Alkyl Phenols (nonionic):

Alkyl chains of 8 to 20 carbons, usually between 4 and 14 carbons and more preferred to be 8 or 9 carbons, with 4-20 moles of ethylene oxide, usually between 7 25 and 20 moles and more preferred to 8-12 moles.

Examples: Nonylphenol with 9 moles ethylene oxide, octylphenol with 8 moles ethylene oxide.

8. Sulfates or Sulfonates of Ethoxylated Alkyl Phenols (and their salts) (anionic)

Examples: Nonyl phenol sulfate or sulfonate with 9 moles ethylene oxide; octyl phenol sulfate or sulfonate with 8 moles ethylene oxide.

9. Fluorocarbon-based Surfactants (nonionic, amphoteric, anionic):

These must be water-soluble forms. Fluorocarbon esters such as 3M Company's "FC-74" are oil soluble and not appropriate for this use. 3M Company's "FC-100", "C-129", "FC-170C" are commercially available examples of fluorocarbon-based surfactants used in the 40 invention.

Examples: Fluoro-octyl sulfonate or sulfate, perfluorinated quaternary ammonium oxide, and fluorinated C<sub>9</sub>-C<sub>11</sub> alcohols with 7 moles ethylene oxide.

10. Phosphate Derivatives of Ethoxylated Alcohols: 45

Examples: C<sub>14</sub>-C<sub>16</sub> linear alcohols phosphate with 8 moles ethylene oxide; phosphated nonylphenol with 10 moles ethylene oxide.

11. Quaternary Ammonium Chloride (cationic):

Dimethyl dicoco ammonium chloride, cetyl dimethyl 50 benzyl ammonium chloride, cetyl dimethyl ammonium chloride.

12. Sulfates or Sulfonates of Alcohols (and their salts) (Anionic):

Sulfated simple alcohols with carbon chains of 8-20, 55 usually between 10 and 16 and most common 10-12.

Examples: Sodium lauryl sulfate or sulfonate, potassium lauryl sulfate or sulfonate, magnesium lauryl sulfate or sulfonate, sodium n-decyl sulfate or sulfonate, triethanol amine lauryl sulfate or sulfonate, sodium 2-ethylhexyl sulfate or sulfonate.

13. Condensation Products of Ethylene Oxide and Propylene Glycol (nonionic):

Examples: Propoxylated C<sub>9</sub>-C<sub>11</sub> alcohols with 6 moles ethylene oxide.

The surfactants or mixtures of surfactants should be soluble in the cementitious slurry and not precipitate or otherwise degrade under the action of the ions in the

cementitious slurry (e.g., resistant to calcium and other electrolytes) and the temperature and pressure conditions occurring during the placement and curing of the cement.

- 5 Especially preferred are nonylphenol ethoxylates, coco amido betaine, blends of N-alkyl coco trimethyl ammonium chloride and bis(2-hydroxyethyl) cocoamide oxide, blends of ethoxylated trimethylolnonanol and perfluoro quaternary ammonium oxide, C<sub>12</sub>-C<sub>15</sub> linear 10 alcohol ethoxylate sulfate, C<sub>9</sub>-C<sub>11</sub> linear alcohol ethoxylate sulfates, sodium lauryl sulfate, and ethoxy alcohol sulfates.

The concentration of surfactant in the water phase used to prepare the slurry will generally be from about 0.1 to about 5% by weight, and more preferably from about 0.2 to about 3% by weight; excellent results have been obtained with concentrations between about 1.17 and about 2.33% by volume.

## ALCOHOLS

The invention is very effective for solidification of drilling fluids containing polyhydric alcohols. The following alcohols may be used alone or in blends with the preceding surfactants. The polyalcohol ingredients of drilling fluids containing polyalcohols are preferably acyclic polyols having at least two carbon atoms and 2 hydroxyl groups but no more than 18 carbon atoms and 13 hydroxyl groups. Preferably, the polyols of the invention have at least 2 carbon atoms and 2 hydroxyl groups, but no more than 9 carbon atoms and 7 hydroxyl groups.

Nonlimiting examples of such polyols include (carbons chains may be straight or branched), ethylene glycol, diethylene glycol, 1,2-propanediol, 1,3-propanediol (propylene glycol), neopentyl glycol, pentaerythritol, 1,6-hexanediol, glycerol, telomers of glycerol such as diglycerols, triglycerols, tetraglycerols, pentaglycerols, and hexaglycerols, mixtures of glycerol and telomers of glycerol such as diglycerol and triglycerols, mixtures of telomers of glycerol, polyethylene glycols, polypropylene glycols, ethylenepropylene glycol, polyethylenepropylene glycols, ethylene-propylene glycol copolymers and ethylenebutylene glycol copolymers, 1,5,6,9-decanetetrol, 1,1,4,4-cyclohexanetetramethanol, 1,2,4,5-cyclohexanetetramethanol, 1,4-cyclohexanediethanol, 1,3-cyclopentanediethanol, 1,2,4,7-heptanetetrol, 1,2,3,5-heptanetetrol, 1,5,8-nanetriol, 1,5,9-nanetriol, 1,3,5,9-nanonetrol, 1,3,5-heptanetriol, 2,4,6-heptanetriol, 4,4-dimethyl-1,2,3-pentanetriol, 1,1,3-cyclohexanetriethanol, 1,3,4-cycloheptanetriol, 1,1-cyclopropanediol, 1,2-cyclopropanediol, 1,2,3-cyclopropanetriol, 1,1-cyclopropanedimethanol, 2,2-cyclopropanedimethanol, 1,2,3-cyclopropanedimethanol, 1,1-cyclobutanediol, 1,2-cyclobutanediol, 1,3-cyclobutanediol, 1,2-cyclobutanedimethanol, 1,2,3-cyclobutanetriol, 1,2,4-cyclobutanetriol, 1,2,3,4-cyclobutanetetrol, 1-hydroxycyclobutanemethanol, 3-methyl-2,2-butanediol, 1,2-pantanediol, 1,3-pantanediol, 1,4-pantanediol, 2,3-pantanediol, 2,4-pantanediol, 1,2,3-pantanetriol, 1,2,4-pantanetriol, 2,3,4-pantanetriol, 1,1-cyclopantanediol, 1,2-cyclopantanediol, 1,3-cyclopantanediol, 1,2,3-cyclopantanetriol, 1,2-hexanediol, 1,3-hexanediol, 1,2,3-hexanetriol, 1,2,4-hexanetriol, 1,2,3,4-hexanetetrol, 1,1-cyclohexanediol, 1,2-cyclohexanediol, 1,4-cyclohexanediol, 1,2,4-cyclohexanetriol, 1,2,5-cyclohexanetriol, 1,2,3,4-

cyclohexanetetrol, 1,2,3,5-cyclohexanetetrol, sorbitol, mannitol.

More preferred alcohols are cyclicetherpolyols having at least 6 carbon atoms, at least 2 hydroxyl groups, and at least 2 ether linkages. Even more preferred are 5 cyclicetherpolyols having at least 15 carbon atoms, 5 ether linkages, and at least 2 hydroxyl groups, or at least 15 carbon atoms, at least 7 ether linkages, and at least 3 hydroxyl groups. Most preferred are cyclicetherpolyols having at least 18 carbon atoms, at least 6 hydroxyl groups, and at least 6 ether linkages. Molecular structures with significantly larger molecular weights than the above minimums have been found to be advantageous. Among the cyclicetherpolyols, monocyclicdetherdiols are preferred and polycyclicpolyetherpolyols (referred to hereinabove as PECP) are most preferred. "Poly" is used to mean two or more.

The alcohols or mixtures of alcohols useful in this invention should be soluble in the drilling fluid of this invention at the temperature and pressure conditions occurring in the wellbore or can be solubilized as described infra. Additionally, the alcohols or mixtures of alcohols should not precipitate or otherwise degrade under the actions of the ions in the drilling fluid (e.g., 20 resistant to calcium and electrolytes) and the temperature and pressure conditions occurring during drilling. The alcohols may also be soluble at the ambient temperature and pressure conditions on the surface during the preparation of the drilling fluid of this invention. Some of the higher molecular weight alcohols may be very 25 viscous liquids, or solids or have low solubility at the temperature conditions at the surface under which the drilling fluid is prepared. In these cases, the alcohols may be diluted with a suitable solvent which is soluble in the drilling fluid at the temperature conditions of drilling fluid preparation at the surface. Such suitable solvents may act to both lower viscosity and to increase 30 solubility of the higher molecular weight alcohol for addition to the drilling fluid on the surface. Such solvents may be polyols of lower molecular weight, other alcohols such as methanol, ethanol, propanol, or isopropanol, water or mixtures of solvents and water.

The concentration of alcohol in the water phase when used in the preparation of the drilling fluid of this invention will generally be at least about 2% by weight and preferably from about 2 to about 30% by weight based on the water phase and more preferable from about 5 to about 15% by weight; excellent results have been obtained with concentrations between about 10 and about 20% by weight. Preferably at least about 1% w of the alcohol is cyclicetherpolyol or acyclic polyol, based on the total weight of the alcohol.

Example 1 The following examples demonstrate the disadvantages of using Portland cement for cement 55 plugs.

TABLE 1

| Effect of Drilling Fluid Contamination on Portland Cement Thickening Time      |                                        |                             |
|--------------------------------------------------------------------------------|----------------------------------------|-----------------------------|
| Drilling Fluid Type                                                            | Cement:Drilling Fluid Volumetric Ratio | Thickening Time Hours       |
| Test Temperature:<br>172° F.                                                   |                                        |                             |
| Oil external emulsion - with 30% (bw) calcium chloride brine as internal phase | 100:0<br>95:5<br>75:25<br>50:50        | 4.38<br>3.65<br>1.98<br>1.8 |

TABLE 1-continued

| Effect of Drilling Fluid Contamination on Portland Cement Thickening Time |                                        |                       |
|---------------------------------------------------------------------------|----------------------------------------|-----------------------|
| Drilling Fluid Type                                                       | Cement:Drilling Fluid Volumetric Ratio | Thickening Time Hours |
| Test Temperature:<br>150° F.                                              |                                        |                       |
| Water base                                                                | 100:0                                  | 4.23                  |
| Lignosulfonate                                                            | 95:5<br>75:25<br>50:50                 | 5.66<br>6.5+<br>8+    |

TABLE 2

| Effect of Drilling Fluid Contamination on Compressive Strength of Portland Cement |                                        |                             |
|-----------------------------------------------------------------------------------|----------------------------------------|-----------------------------|
| Drilling Fluid Type                                                               | Cement:Drilling Fluid Volumetric Ratio | Compressive Strength, psi   |
| Test Temperature:<br>250° F.                                                      |                                        |                             |
| Oil external emulsion - with 30% (bw) calcium chloride brine as internal phase    | 100:0<br>90:10<br>75:25                | 2514<br>2230<br>660         |
| Test Temperature:<br>175° F.                                                      |                                        |                             |
| Water base                                                                        | 100:0                                  | 3275                        |
| Lignosulfonate                                                                    | 95:5<br>75:25<br>50:50                 | 2670<br>1680<br>did not set |

TABLE 3

| Effect of Drilling Fluid on Shear Bond Between Portland Cement and a Steel Surface |                         |
|------------------------------------------------------------------------------------|-------------------------|
| Coating Material on Surface of Steel Rod                                           | Shear Bond Strength psi |
| None - Clean steel surface                                                         | 170                     |
| Water base drilling fluid                                                          | 55                      |
| Water base spacer fluid                                                            | 80                      |
| Oil base drilling fluid                                                            | 5                       |
| Oil base spacer fluid                                                              | 25                      |

## EXAMPLE 2

Base Mud: Fresh water mud containing bentonite, chrome lignosulfonate, and low viscosity polyanionic cellulose.

300 lbs of hard burned magnesium oxide, under the trade name of "MAGCHEM 10 CR" by Martin Marietta Magnesia Specialties was added to weight the base mud up to 12.6 lbs/gal. Varying amounts of an ammonium polyphosphate solution were added to solidify the mud. The ammonium polyphosphate solution used is "POLY-N" sold by Arcadian Corporation and contains about 50 wt % ammonium polyphosphate. The results are described in the following table.

| 60 | Amount of Poly-N Added, % by volume of the mud | Resulting Density lbs/gal | Description of the resulting solid   |
|----|------------------------------------------------|---------------------------|--------------------------------------|
| 65 | 0                                              | 12.6                      | Did Not Set                          |
|    | 25                                             | 12.4                      | Set, resilient                       |
|    | 50                                             | 12.3                      | 50 psi after 4 hrs<br>Set, resilient |
|    | 100                                            | 12.2                      | 40 psi after 4 hrs<br>Set, resilient |

-continued

| Amount of Poly-N<br>Added, % by volume<br>of the mud | Resulting<br>Density<br>lbs/gal | Description of<br>the resulting<br>solid |
|------------------------------------------------------|---------------------------------|------------------------------------------|
|                                                      |                                 | 30 psi after 4 hrs                       |

This example shows that solutions of polyphosphates can be used as diluents while also converting the drilling fluid into a solid.

## EXAMPLE 3

Base Mud: Fresh water mud containing bentonite, chrome lignosulfonate, and low viscosity polyanionic cellulose.

300 lbs of hard burned magnesium oxide, under the trade name of "MAGCHEM 10 CR" by Martin Marietta Magnesia Specialties was added to weight the base mud up to 12.6 lbs/gal. Varying amounts of a monoammonium phosphate were added to solidify the mud. The results are described in the following Table.

| Amount of MAP<br>Added, % by wt of MgO<br>of the mud | Resulting<br>Density<br>lbs/gal | Description of<br>the resulting<br>solid |
|------------------------------------------------------|---------------------------------|------------------------------------------|
| 0                                                    | 12.6                            | Did Not Set                              |
| 25                                                   | 12.6                            | Set, resilient<br>50 psi after 4 hrs     |
| 50                                                   | 12.7                            | Set, resilient<br>250 psi after 2 hrs    |
| 100                                                  | 12.85                           | Set, hard<br>510 psi after 2 hrs         |

## EXAMPLE 4

Base Mud: Fresh water mud containing bentonite, chrome lignosulfonate, and low viscosity polyanionic cellulose.

300 lbs of hard burned magnesium oxide, under the trade name of "MAGCHEM 10 CR" by Martin Marietta Magnesia Specialties was added to weight the base mud up to 12.6 lbs/gal. Varying amounts of a polyacrylic acid solution were added to solidify the mud. The polyacrylic acid had an average molecular weight of about 20,000 and is sold by PolySciences, Inc. The solution contained about 40 wt % polyacrylic acid. The results are described in the following Table.

| Amount of Polyacrylic<br>Acid Added, % by<br>volume of the mud | Resulting<br>Density<br>lbs/gal | Description of<br>the resulting<br>solid                               |
|----------------------------------------------------------------|---------------------------------|------------------------------------------------------------------------|
| 0                                                              | 12.6                            | Did Not Set                                                            |
| 25                                                             | 11.9                            | Set, resilient<br>good adhesion to surfaces<br>40 psi after 4 hrs      |
| 50                                                             | 11.5                            | Set, resilient<br>good adhesion to surfaces<br>40 psi after 4 hrs      |
| 100                                                            | 10.9                            | Set, highly pliable<br>good adhesion to surfaces<br>10 psi after 4 hrs |

This Example shows that solutions of functional group-containing polymers can be used as diluents while also converting the drilling fluid into a solid.

## EXAMPLE 5

Base Mud: Fresh water mud containing bentonite, chrome lignosulfonate, and low viscosity polyanionic cellulose.

300 lbs of hard burned zinc oxide, prepared in the laboratory by heating analytical grade zinc oxide at 1350° C. for 8 hours, cooling and grinding to pass through a 325 mesh screen, was added to weight the base mud up to 13.5 lbs/gal. Varying amounts of a polyacrylic acid solution were added to solidify the mud. The polyacrylic acid had an average molecular weight of about 50,000 and is sold by PolySciences, Inc. The solution contained about 25 wt % polyacrylic acid. The results are described in the following Table.

| Amount of Polyacrylic<br>Acid Added, % by<br>volume of the mud | Resulting<br>Density<br>lbs/gal | Description of<br>the resulting<br>solid |
|----------------------------------------------------------------|---------------------------------|------------------------------------------|
| 0                                                              | 13.5                            | Did Not Set                              |
| 100                                                            | 11.3                            | Set, ductile<br>310 psi after 4 hrs      |

## EXAMPLE 6

Base Mud: Fresh water mud containing bentonite, chrome lignosulfonate, and low viscosity polyanionic cellulose.

300 lbs of hard burned magnesium oxide, under the trade name of "MAGCHEM 10 CR" by Martin Marietta Magnesia Specialties was added to weight the base mud up to 12.6 lbs/gal. Varying amounts of ethylene/acrylic acid copolymers were added by weight of the magnesium oxide. The copolymers used were "ACLYN" 540, 580, and 5120 sold by Allied Signal, Inc. These copolymers have low molecular weights and varying amounts of acrylic acid incorporated into the polymer. AC 540 has the lowest acrylic acid content and AC 5120 has the highest acrylic acid content.

Each mixture was heated to a temperature above the melting point of the copolymer and held at that temperature for 24 hours. The average melting point temperature for each of these copolymers was about 100° C. After 24 hours the samples were cooled and extracted from the molds. Each had set to form a cohesive solid having compressive strengths between 50 and 700 psi. All samples were ductile and good adhesion to metal surfaces.

## EXAMPLE 7

Base Mud: Fresh water mud containing bentonite, chrome lignosulfonate, and low viscosity polyanionic cellulose.

350 lbs of blast furnace slag sold under the trade name of "NEWCEM" by Blue Circle Cement Company was added to weight the mud to lbs/gal. An equal volume amount of a polyacrylic acid solution were added to solidify the mud. The polyacrylic acid had an average molecular weight of about 50,000 and is sold by PolySciences, Inc. The solution contained about 25 wt % polyacrylic acid. The results are described in the following Table.

| Amount of Polyacrylic<br>Acid Added, % by volume<br>of the mud | Resulting<br>Density<br>lbs/gal | Description of<br>the resulting<br>solid |
|----------------------------------------------------------------|---------------------------------|------------------------------------------|
| 0                                                              | 12.6                            | Did Not Set                              |

-continued

| Amount of Polyacrylic<br>Added, % by volume<br>of the mud | Resulting<br>Density<br>lbs/gal | Description of<br>the resulting<br>solid |
|-----------------------------------------------------------|---------------------------------|------------------------------------------|
| 100                                                       | 10.9                            | Set, ductile<br>130 psi after 4 hrs      |

**What is claimed is:**

1. A method for restoring drilling fluid circulation to a borehole of a well having surrounding strata being invaded by the drilling fluid which is thereby escaping the borehole, comprising:

### preparing a cementitious slurry comprising:

- (a) a cementitious component selected from granulated water-quenched blast furnace slag and a proton acceptor metal compound and
  - (b) an activator wherein, when said cementitious component is said blast furnace slag, said activator is optionally an alkaline agent, and when said cementitious component is said metal compound, said activator is a phosphorus acid or one of a polymer component of the formula:



wherein A is



or a mixture of



and wherein R is H or a 1-10 carbon atom alkyl radical and the ratio of m to n is within the range of 50:1 to 100:1; and

- (c) a water source selected from water, brine, seawater, water base drilling fluid, and water emulsion drilling fluid; displacing the cementitious slurry into the strata 55 which the first said drilling fluid is invading, the

cementitious slurry being in direct contact, during and after placement, with the drilling fluid in the borehole; and allowing the cementitious slurry to solidify in situ to form a plug in the wellbore and thereby sealing the strata from the wellbore.

2. The method of claim 1 wherein the wellbore is subsequently reopened by drilling through the plug.
  3. The method of claim 1 wherein the borehole is drilled with a universal fluid containing a minor quantity of the cementitious component, and a settable filter cake is deposited on the wall of the borehole.
  4. The method of claim 3 wherein the well is cemented by adding a major quantity of the cementitious component to the universal fluid.
  5. The method of claim 1 wherein the cementitious slurry is a blend including more than one of the cementitious components.
  6. The method of claim 1 wherein the cementitious slurry is a blend including more than one of the cementitious components and more than one of the activators.
  7. The method of claim 1 wherein the cementitious component is the blast furnace slag and the activator is the alkaline agent.
  8. The method of claim 1 wherein the cementitious component is the proton acceptor metal compound and the activator is the phosphorus acid.
  9. The method of claim 1 wherein the cementitious component is the proton acceptor metal compound and the activator is the polymer compound.

10. The method of claim 1 wherein the cementitious component is the proton acceptor metal compound, and the activator is the polymer compound and the phosphorus acid.
11. The method of claim 1 wherein the cementitious component is the blast furnace slag, and the activator is the alkaline agent and the polymer component.

- 40 12. A method for restoring drilling fluid circulation to a borehole of a well having surrounding strata being invaded by the drilling fluid which is thereby escaping the borehole, comprising:

45 preparing a cementitious slurry comprising: granulated water-quenched blast furnace slag and a water source selected from the group consisting of water, brine, seawater, water base drilling fluid, and water emulsion drilling fluid;

50 displacing the cementitious slurry into the strata which the first said drilling fluid is invading, the cementitious slurry being in direct contact, during and after placement, with the drilling fluid in the borehole; and

55 allowing the cementitious slurry to solidify in situ to form a plug in the well bore and thereby seal the strata from the wellbore.

本 本 本 本 本